

## 1

2,929,778

## CORROSION RESISTANT SULFURIZED-PHOSPHORIZED EXTREME PRESSURE LUBRICANT

Allan A. Manteuffel, Crystal Lake, George W. Ayers, Chicago, and William D. Gilson, Crystal Lake, Ill., assignors to The Pure Oil Company, Chicago, Ill., a corporation of Ohio

No Drawing. Application September 13, 1956  
Serial No. 609,543

7 Claims. (Cl. 252—24)

This invention relates to lubricants and to lubricant additives, and more particularly to extreme pressure lubricants and to additives capable of imparting to mineral and other lubricating oils high load-carrying ability, and to their method of manufacture.

The use of chlorine-, sulfur-, and phosphorus-containing compositions as E.P. lubricant additives is well known. Each type of additive has its advantages and disadvantages. The halogen-containing additives, while capable of imparting high load-carrying characteristics to oils, have the disadvantage of being corrosive and hydrolyzing in service to form objectionable acids. The ability of sulfur to impart high load-carrying characteristics to a lubricating oil is dependent on the activity of the sulfur, which in turn is dependent on the tightness with which it is chemically bound in a compound. Elemental or loosely bound sulfur, while imparting high load-carrying characteristics, is too corrosive to be allowed to remain in an automotive differential or other gear assembly over a long period of time. The same is true of the phosphorus sulfides. On the other hand, sulfur and phosphorus sulfides when tightly bound chemically to organic compounds such as fatty acids, fatty esters, fatty alcohols and terpenes, impart excellent load-carrying characteristics to a lubricating oil and are substantially non-corrosive. However, additives of this type will not give the desired protection against wear to new gears during the initial break-in period.

An object of this invention is to provide an extreme pressure lubricant. Another object of this invention is to provide a composition which can be added to mineral and other lubricating oils to impart thereto extreme pressure characteristics. A further object of the invention is to provide a lubricant which will protect gears against wear during the initial break-in period and during the subsequent running life of the gears. Still another object of the invention is to provide a composition which can be added to mineral oil and other types of lubricants to enable such lubricants to satisfactorily lubricate automotive gears during the initial break-in period and during the subsequent running life thereof. A still further object of the invention is to provide an extreme pressure lubricant which will satisfactorily lubricate gear assemblies during the initial break-in period and during the subsequent running life thereof without causing undue corrosion of the gear elements. Still another object is to provide a method for making the aforesaid compositions and lubricants.

Other objects of the invention will become manifest from the following detailed description of the invention.

In co-pending application Serial No. 606,585 there is disclosed a lubricating oil composed of a major portion of mineral lubricating oil, sulfurized and phosphorized fatty material and free sulfur or sulfur-liberating compound, with or without materials which will accelerate the chemical fixation of the free sulfur, namely, naph-

## 2

thenate salts and ammonium or amine salts of sulfonic acids. We have discovered that the conversion of the active sulfur to a non-corrosive form can be accelerated by incorporating in the oil a small amount of an organic phosphite or trithiophosphite (also called a phosphorotriethioite). The accelerators used in accordance with our invention may be represented by the general formula  $(RS)_3P$  (phosphorotriethioites) and  $(RO)_3P$  (phosphites) in which the R may be an alkyl, aryl or alkylaryl radical.

As specific examples of compounds falling within the scope of this invention may be mentioned triethyl phosphorotriethioite, diethyl hydrogen phosphite, and tricresyl phosphite. Any alkyl, aryl or alkylaryl phosphite or phosphorotriethioite may be used which is sufficiently soluble in the finished oil so that it does not precipitate out during storage.

The phosphites and phosphorotriethioites are effective for rendering sulfur non-corrosive, either in the presence or absence of naphthenate salts. In order to improve the anti-weld properties of lubricants in accordance with our invention, we prefer to incorporate into the lubricant blend a naphthenate salt such as lead naphthenate. The sulfurized-phosphorized fatty material, sulfur and lead naphthenate cooperate to provide the required anti-weld properties to the lubricant during the break-in period and the sulfurized-phosphorized fatty material in conjunction with dibenzyl disulfide imparts the required load-carrying properties to the oil during operation subsequent to the break-in period.

As sulfurized and phosphorized compositions which are effective for the purpose of our invention we prefer sulfurized and phosphorized fatty bodies such as those made in accordance with Whittier et al., Patent 2,211,306. As therein disclosed, such sulfurized and phosphorized fatty bodies are prepared by sulfurizing a fatty material such as vegetable, animal, or marine oils and waxes, including but not limited to wool grease, cotton seed, castor, rape seed, sperm and lard oils, and synthetic esters of high molecular weight, mono-unsaturated fatty acids ( $C_{16}$ — $C_{24}$ ), such as glyceryl trioleate, propylene glycol dioleate and butylene glycol dioleate, at a temperature of approximately 330—340° F. with elemental sulfur until a satisfactory copper strip test is obtained, and then phosphorizing the sulfurized material with a phosphorus sulfide, preferably phosphorus sesquisulfide, at a temperature of about 220—230° F. until a satisfactory copper strip is obtained.

Instead of following the process set forth in the aforesaid Whittier et al. patent, the initial sulfurization step may be terminated prior to the time a satisfactory copper strip test is obtained, that is, when the copper strip shows a tan color, and then phosphorized with a phosphorus sulfide for a sufficiently long period of time to more firmly bind the sulfur and phosphorus. This method is particularly effective where higher amounts of phosphorus sesquisulfide within the limits of those disclosed in the aforesaid patent are used in the phosphorization step. As a specific example, lard oil was mixed with 7.5% of sulfur and then was stirred with constant agitation in a kettle at a temperature of 325—340° F. Heating was continued for approximately four hours, at which time the copper strip gave a tan color upon immersion in a sample of the product at 300° F. for one minute. The mixture was then rapidly cooled to approximately 220° F., 0.8% by weight of phosphorus sesquisulfide was slowly added in finely divided form, and the reaction was allowed to continue at 220—230° F. for a period of eight hours, after which the mixture was rapidly cooled to 120° F. and thereafter allowed to cool to room temperature. The final product contained 7.85% sulfur and 0.45% phos-

phorus by weight and gave a tan color on the copper strip test at 220° F. for one minute.

In preparing sulfurized-phosphorized fatty materials in accordance with the method just described, the fatty material may be reacted with about 5 to 10% of sulfur in the first stage and with from about 0.4 to 5% of phosphorus sesquisulfide or equivalent amount of other phosphorus sulfide in the second stage. This method of preparing sulfurized-phosphorized fatty materials, in which sulfur is not tightly bound in the first stage and relatively large amounts of phosphorus sulfide are reacted in the second stage, is disclosed and claimed in co-pending application of P. R. Chapman and A. Manteuffel, Serial No. 553,419.

Instead of using elemental sulfur in conjunction with the sulfurized-phosphorized fatty material, we may add to the oil an unstable sulfur compound which will release elemental sulfur as, for example, dibenzyl trisulfide or other alkyl, aryl or arylalkyl polysulfides containing three or more sulfur atoms in the molecule. A phosphorus sulfide such as phosphorus sesquisulfide suspended or dissolved in the mineral oil will also function to provide the anti-weld properties for which the elemental sulfur is added. If desired, both sulfur and a phosphorus sulfide such as phosphorus sesquisulfide may be used in combination within the limits of the amounts specified above for sulfur. If a sulfur-liberating compound is used, it should be added in amounts sufficient to liberate the desired amount of sulfur.

In preparing gear oils in accordance with our invention, the sulfur or active sulfur-containing compound is dissolved in a portion or all of the mineral oil at a temperature of about 270-290° F. After the addition of the sulfur or active-sulfur compound is complete, the temperature of the oil is reduced to about 200° F. before adding the sulfurized-phosphorized fatty material. It is important to reduce the temperature to this level to avoid immediate or rapid reaction, inactivation, or absorption of the sulfur into a substantially less active form. A suitable temperature for admixture of the sulfur-containing oil and the sulfurized-phosphorized fatty body is about 160-200° F.

The manner of mixing the several constituents together or the order in which they are admixed is not important, provided temperatures are properly adjusted to a level which will permit solution of the additives in the oil within a reasonable period of time without causing substantial reaction between the active sulfur and the sulfurized-phosphorized fatty material. The sulfurized-phosphorized fatty material, dibenzyl disulfide, naphthenate salt and phosphite or phosphorothioite, as well as other additives such as pour point depressors, V.I. improvers and anti-foam agents, may be added separately to the oil or may be admixed together and added as an admixture. They may be dissolved directly in the oil in which the sulfur or active-sulfur compound which has been previously dissolved, or they may be admixed with a portion of the oil to which the sulfur or active-sulfur compound has not been added and this portion added to the portion containing the sulfur or active-sulfur compound. We prefer to add dibenzyl disulfide or equivalent disulfide as disclosed in claims in Reissue Patent 22,911, in order to improve the load-carrying properties of the oil. We also, preferably, incorporate in the finished lubricant a sufficient amount of aromatic extract obtained in the solvent extraction of mineral lubricating oil fractions by means of phenol, fufural, nitrobenzene and equivalent solvents in order to prevent precipitation.

In order to realize the benefits of our invention, it is necessary to adjust the proportions of sulfurized-phosphorized fatty material and sulfur, or active-sulfur compound, so that the active sulfur is absorbed or chemically bound by the sulfurized-phosphorized material and does not remain in the oil in a corrosive form over a long period of time. If the ratio of sulfur or active-sulfur

fur compound to sulfurized-phosphorized fatty material is too high, the sulfur will not be completely absorbed and the corrosive condition of the gear oil will continue for an indefinite period of time with resultant harmful wear of the gear parts. The amount of sulfur which can be chemically absorbed is determined by the amount of the sulfurized-phosphorized fatty material and phosphite or phosphorothioite present and also by the amount of sulfur bound in the sulfurized-phosphorized material. A 5 sulfurized-phosphorized material containing a relatively low amount of bound sulfur, as, for example, 5% by weight, enables the use of a larger amount of free sulfur or active sulfur-containing material than does a sulfurized-phosphorized material containing a higher amount 10 as, for example, 10% of bound sulfur. In general, we have found that an amount of sulfur or equivalent active sulfur-containing compound between 1 and 50% of the quantity of sulfurized-phosphorized fatty material is effective in providing initial anti-weld characteristics to the 15 oil during the break-in period and of being subsequently absorbed or reacted with the sulfurized-phosphorized fatty material to a substantially non-corrosive state. We prefer an amount of sulfur equivalent to about 3 to 10% by weight of the sulfurized-phosphorized fatty material.

20 The amount of free sulfur or active sulfur-containing material to be added will be determined to some extent by the nature of the gears to be lubricated. For example, in the case of phosphate-coated gears the number of miles required for breaking them in is probably not more than 25 25 30 35 40 45 50 55 60 65 70 75

100 and may be as low as 25 to 50. In such cases, therefore, it may be desirable to incorporate smaller amounts of sulfur so that the sulfur will be bound in an inactive or non-corrosive form within a short period of time, probably not more than 24 hours. On the other hand, "green gears," that is, gears which are not precoated, are usually considered to be broken in after 500 miles of recommended driving speed. In such cases, sufficient sulfur should be present so that it will not be completely bound before the end of the period required to drive 500 miles, which on an average may be approximately one week.

The amount of sulfur required in the oil to furnish anti-weld protection during the necessary period of break-in can be approximated by subjecting an oil blend maintained at approximately 200° F. for the requisite period of time to the copper strip test, performed by immersing a clean copper strip for three minutes in a sample of the oil maintained at a temperature of 210° F. The appearance of the strip after this test provides an indication of the amount of corrosion which occurred and hence the extent to which the active sulfur has been bound in a non-active form. If the color of the strip remains clear and bright it is indicative of the fact that the sulfur has been tightly bound chemically and is in non-corrosive form. As the color of the strip progresses through light orange, orange, light brown, medium brown, mottled brown and brown-black, it indicates that the oil is more and more corrosive.

In order to demonstrate the effectiveness of compositions made in accordance with our invention, a number of blends were prepared and subjected to the copper strip corrosion test. The blends tested and the corrosion tests on each blend are given in the following table. Blends were made by dissolving free sulfur in approximately half of the total mineral oil, previously blended, at a temperature of 270-290° F. with stirring. The total mineral oil consisted of a blend of mineral oil, bright stock and solvent extract. These three constituents were blended together to give the desired finished viscosity and V.I. The extract oil was used to insure complete compatibility of the additives, particularly sulfurized-phosphorized lard oil, in the finished oil and to inhibit precipitation.

After the sulfur had been dissolved in a portion of the mineral oil, the remainder of the oil was added, resulting 75 in cooling of the solution to below 200° F. Sulfurized-

phosphorized lard oil, dibenzyl disulfide, lead naphthenate and phosphite or phosphorotriethioite were then added as indicated in the specific blends. During the addition of these additives, the oil was at a temperature between 160° F. and 200° F. The temperature was maintained below 200° F. to avoid premature inactivation of the sulfur.

Portions of the blends were heated in an oil bath to 200° F. and samples were subjected to the three-minute copper strip test at 210° F. after reaching bath temperature and thereafter at intervals of one hour, two hours, twenty-four hours, and one week. The temperature of 200° F. was selected as representing the average temperature to which gear oils are subjected in service. The sulfurized and phosphorized lard oil used in the blends given in the ensuing table was made by heating 91.7 parts by weight of lard oil to 285°, plus or minus 10° F., and then dusting in slowly, with agitation, 7.5 parts by weight of sulfur. After the addition of the sulfur the temperature was raised to 335°, plus or minus 5° F., and held at that level for four hours. At the completion of the heating period a copper strip was immersed in the bath for three minutes and was only lightly tarnished. The temperature of the reaction mixture was then lowered to 220°, plus or minus 5° F., and 0.8 part by weight of phosphorus sesquisulfide was slowly added. This temperature level was maintained for eight hours with continuous mechanical agitation of the reaction mixture. At the end of this period a copper strip immersed in the bath at 220° F. for three minutes gave a pink coating, indicating that the reaction was completed. The final product contained 7.85% sulfur and 0.45% phosphorus by weight.

From an examination of the table, the following conclusions can be drawn: (1) Blend 1 demonstrates that in the absence of a phosphite or phosphorotriethioite the blend still contained corrosive sulfur after being main-

of the corrosive sulfur and to increase the anti-weld properties of the blend during the break-in period.

The amount of sulfurized and phosphorized fatty material in the blend may range from about 5 to 20% by weight and the amount of dibenzyl disulfide which may be used in the blends may vary within the limits disclosed in Reissue Patent 22,911, but preferably between 0.5 and 2%. The amount of naphthenate salt effective to accelerate the sulfur reaction with the sulfurized-phosphorized lard oil may vary between approximately 0.1 and 5% by weight of the gear oil blend. The amount of phosphorotriethioite and/or phosphite required to accelerate the reaction will be dependent on the particular compound chosen, the amount of active sulfur present and the desired rate of sulfur inactivation. In general, amounts between 0.1 and 5% of the total gear oil blend are effective.

The amount of solvent extract in the blend may vary from 0 to 100% of the mineral oil portion, depending upon the desired V.I. and the compatibility characteristics of the finished blend. In general, amounts from 5 to 30% will prevent precipitation and at the same time give an oil with a commercially desirable V.I. The solvent extract used in the blends reported in the foregoing table had the following characteristics:

|                                   |        |
|-----------------------------------|--------|
| Gravity (° A.P.I.)                | 13.2   |
| Flash (C.O.C., ° F.)              | 550    |
| Fire (C.O.C., ° F.)               | 640    |
| S.U.S. viscosity at 100° F.       | 34,000 |
| S.U.S. viscosity at 150° F.       | 2,824  |
| S.U.S. viscosity at 210° F.       | 404    |
| Viscosity index                   | 17     |
| Pour point (° F.)                 | +65    |
| Total sulfur (percent)            | 2.39   |
| Neutralization number (ASTM D974) | 2.8    |
| Conradson carbon residue          | 4.2    |

Table I

| Composition in parts by weight of gear oil              | Blend No.   |                  |              |                  |                  |
|---------------------------------------------------------|-------------|------------------|--------------|------------------|------------------|
|                                                         | 1           | 2                | 3            | 4                | 5                |
| Neutral Oil, 200 SUS viscosity at 100° F., 90 V.I.      | 46.7        | 46.7             | 46.7         | 46.7             | 46.7             |
| Bright stock, 160-170 SUS viscosity at 212° F., 90 V.I. | 22.0        | 22.0             | 22.0         | 22.0             | 22.0             |
| Solvent Extract                                         | 18.0        | 18.0             | 18.0         | 18.0             | 18.0             |
| Sulfur                                                  | 0.3         | 0.3              | 0.3          | 0.3              | 0.3              |
| Sulfurized-phosphorized lard oil                        | 9.0         | 9.0              | 9.0          | 9.0              | 9.0              |
| Dibenzyl disulfide                                      | 0.8         | 0.8              | 0.8          | 0.8              | 0.8              |
| Lead naphthenate (30-90 Pb)                             | 4.0         | 4.0              | 4.0          | 4.0              | 4.0              |
| Triethyl phosphorotriethioite                           |             |                  |              |                  |                  |
| Diethyl hydrogen phosphite                              |             |                  |              |                  |                  |
| Tricresyl phosphite                                     |             |                  |              |                  |                  |
| Viscosity:                                              |             |                  |              |                  |                  |
| at 100° F.                                              | 983         | 822              | 871          | 884              | 748              |
| at 130° F.                                              | 493.2       | 348.2            | 364.9        | 365.5            | 322.5            |
| at 210° F.                                              | 85.1        | 78.9             | 80.3         | 83.0             | 76.6             |
| Viscosity Index                                         | 91          | 94               | 91           | 96               | 97               |
| 3 Minute Cu Strip Test:                                 |             |                  |              |                  |                  |
| Upon reaching bath temperature (approx. 1/2 hour).      | brown-black | orange           |              |                  |                  |
| After 1 hr. at 200° F.                                  | do          | do               | do           | do               | do               |
| After 2 hr. at 200° F.                                  | do          | clear and bright | do           | light brown      | do               |
| After 24 hr. at 200° F.                                 | do          | clear and bright | orange       | orange           | orange           |
| After 1 week at 200° F.                                 | light brown | clear and bright | light orange | clear and bright | clear and bright |

tained for one week at 200° F.; (2) blend 2 demonstrates that the addition of 2% of triethyl phosphorotriethioite to blend 1 rendered the sulfur non-corrosive after the blend was maintained at 200° F. for two hours; (3) blend 3 demonstrates that with the addition of only 1% of triethyl phosphorotriethioite the blend was slightly corrosive after one week; (4) diethyl hydrogen phosphite in the amount of 1.3% was effective in rendering the blend non-corrosive after one week, as was also true of 3.3% of tricresyl phosphite.

As was previously pointed out, the phosphorotriethioites and the phosphites are effective for inactivating corrosive sulfur in the absence of naphthenate salt. However, naphthenates such as ammonium, sodium, calcium, lead, may be added to the blend to help accelerate the removal

65 of any solvent extract of high aromaticity (above 50%) obtained by extraction of mineral lubricating oil fractions with solvents selective for separating paraffinic from aromatic hydrocarbons may be used in place of the specific extract used in preparing the blends given in the foregoing table.

We claim as our invention:

70 1. A lubricant composition consisting essentially of mineral lubricating oil, from 5 to 20% by weight of fatty material which has been reacted with 5 to 10% by weight of sulfur and then with 0.4 to 5% by weight of phosphorous sesquisulfide until the product is substantially non-corrosive as measured by the copper strip test, from 0.1 to 5% of sulfur, about 0.5 to 2% by weight of dibenzyl disulfide, and a material from the group con-

sisting of oil soluble alkyl, aryl and arylalkyl phosphites and phosphorotriethioites in an amount of about 0.5 to 4% by weight.

2. A lubricant composition consisting essentially of mineral lubricating oil, from 5 to 20% by weight of lard oil which has been reacted with 5 to 10% by weight of sulfur and then with 0.4 to 5% by weight of phosphorus sesquisulfide until the product is substantially non-corrosive as measured by the copper strip test, from 0.1 to 5% of sulfur, about 0.5 to 2% by weight of dibenzyl disulfide, and a material from the group consisting of alkyl, aryl and arylalkyl phosphites and phosphorotriethioites in an amount of about 0.5 to 4% by weight.

3. Lubricant composition in accordance with claim 2 containing about 0.1 to 5% by weight of lead naphthenate.

4. Lubricant composition in accordance with claim 3 containing sufficient highly aromatic solvent extract from the extraction of mineral lubricating oil to substantially prevent precipitation.

5. Lubricant composition in accordance with claim 4 in which the material is triethyl phosphorotriethioite.

6. Lubricant composition in accordance with claim 4 in which the material is diethyl hydrogen phosphite.

7. Lubricant composition in accordance with claim 4 in which the material is tricresyl phosphite.

References Cited in the file of this patent

UNITED STATES PATENTS

|    |           |           |       |                |
|----|-----------|-----------|-------|----------------|
| 10 | 2,160,577 | Maag      | ----- | May 30, 1939   |
|    | 2,212,899 | Flaxman   | ----- | Aug. 27, 1940  |
|    | 2,382,115 | Stucker   | ----- | Aug. 14, 1945  |
|    | 2,391,311 | Helmore   | ----- | Dec. 18, 1945  |
|    | 2,422,630 | Musselman | ----- | June 17, 1947  |
|    | 2,432,095 | Frey      | ----- | Dec. 9, 1947   |
| 15 | 2,560,542 | Bartleson | ----- | July 17, 1951  |
|    | 2,580,005 | Cyphers   | ----- | Dec. 25, 1951  |
|    | 2,629,721 | Sunde     | ----- | Feb. 24, 1953  |
|    | 2,764,547 | Fields    | ----- | Sept. 25, 1956 |

FOREIGN PATENTS

|    |         |        |       |               |
|----|---------|--------|-------|---------------|
| 20 | 462,553 | Canada | ----- | Jan. 17, 1950 |
|----|---------|--------|-------|---------------|